

## UNITED STATES PATENT OFFICE

CHARLES K. STROBEL, OF PITTSBURGH, PENNSYLVANIA, ASSIGNOR TO THE UNION SWITCH & SIGNAL COMPANY, OF SWISSVALE, PENNSYLVANIA, A CORPORATION OF PENNSYLVANIA

## COPPER OXIDE RECTIFIER

No Drawing.

Application filed June 18, 1930. Serial No. 462,145.

My invention relates to copper oxide rectifiers, and has for an object the provision of a novel and improved method of manufacturing a high resistance rectifier of this type.

I will describe one method embodying my invention, and will then point out the novel features thereof in claims.

In accordance with my invention, a copper blank is first cleaned, and is then placed in an oxidizing furnace maintained at a relatively high temperature, such for example, as 1860° Fahrenheit. It is then removed from such furnace and placed in a second furnace maintained at a lower temperature, such for example, as 1040° Fahrenheit. The oxidized blank is then removed from the second furnace and allowed to cool in still air at room temperature. The blank may be left in the first furnace for approximately 15 minutes, and in the second furnace for approximately 4 minutes.

Heretofore the standard method of producing copper oxide rectifiers has involved heating the copper blank in a first furnace maintained at a relatively high temperature, transferring the oxidized blank to a second furnace maintained at a lower temperature, and then quenching the oxidized blank in water. When produced in this manner, the resistance in the high resistance direction increases with voltage from an initial value at zero volts to a maximum value at about 2 volts, and then decreases with increase of voltage. I have found that when the copper blank is treated in only the first furnace and is then allowed to cool slowly in air, the rectifier has a different voltage-resistance characteristic; in this case, the high resistance increases with voltage up to about 15 volts, and then decreases slowly with increase of voltage. By manufacturing rectifiers in accordance with my present invention, the resistance in the high resistance direction increases with voltage up to about 15 volts, and then decreases slowly with increased voltage in such a manner that the resistance at 30 volts is about the same as the resistance at 2 volts, this resistance value being about 10,000 ohms. The resistance in

the low resistance direction is lower than that of an unquenched rectifier made by the one furnace treatment. Furthermore, an unquenched rectifier made by the two-furnace treatment has an advantage over a rectifier made by the single furnace treatment, in that the aging under load is less severe in the former case than in the latter.

Rectifiers embodying my invention are particularly well adapted for use where high resistance is desirable, such for example, as "B" battery eliminators employed in connection with radio receiving apparatus.

Although I have herein described only one method of rectifier manufacture embodying my invention, it is understood that various changes and modifications may be made therein within the scope of the appended claims without departing from the spirit and scope of my invention.

Having thus described my invention, what I claim is:

1. The method of manufacturing a copper oxide rectifier which consists in placing a copper blank in an oxidizing furnace maintained at substantially 1860° Fahrenheit for 15 minutes, removing the blank from such furnace and placing it in a second furnace maintained at substantially 1040° Fahrenheit for approximately 4 minutes and then removing the oxidized blank and allowing it to cool slowly in still air to room temperature.

2. The method of manufacturing a copper oxide rectifier which consists in heating a copper blank in a furnace maintained at a relatively high temperature, placing the oxidized blank in a second furnace maintained at a lower temperature and then allowing the oxidized blank to cool slowly in still air to room temperature.

In testimony whereof I affix my signature.

CHARLES K. STROBEL